# EUROPEAN PATENT APPLICATION

(11) **EP 4 671 404 A1**
(43) Date of publication of application: **31.12.2025**
(21) Application number: 24184762.3
(22) Date of filing: 26.06.2024
(51) Int. Cl.: C22C 38/04, C22C 38/08, C22C 38/12, C22C 38/06, C22C 38/02, C22C 38/14, C22C 38/00, C21D 9/46, C21D 8/02, C21D 6/00, C21D 6/02, C21D 1/18, C21D 1/22

(54) **LEAN 3RD GENERATION HOT-ROLLED STEEL STRIP AND METHOD OF MANUFACTURING THE SAME**

(71) Applicant: SSAB Technology AB, 101 21 Stockholm (SE)
(72) Inventor: HARJUKELO, Ville, 101 21 Stockholm (SE); KANTANEN, Pekka, 90014 Oulun yliopisto (FI); HANNULA, Jaakko, 90014 Oulun yliopisto (FI); ANTTILA, Severi, 101 21 Stockholm (SE); MEHTONEN, Mikko, 101 21 Stockholm (SE); NOUSIAINEN, Olli, 90014 Oulun yliopisto (FI)
(74) Representative: AWA Sweden AB

(57) **Abstract**

A hot-rolled steel strip, having a yield strength of at least 600 MPa and an ultimate tensile strength of at least 1200 MPa, comprising a composition consisting of, in terms of weight percentages, wt.%:
C 0.15 - 0.4, Mn 1 - 3, Si 0 - 1, Al 0.3 - 1.5, Ni 1 - 3, Mo 0.2 - 1, Ti 0 - 0.2, Nb 0 - 0.1, V 0 - 0.3,
B 0 - 0.005, Ca 0 - 0.006, remainder being Fe and inevitable impurities, wherein P 0 - 0.05, S 0 - 0.01,
N 0 - 0.01, and wherein the sum of Mn and Ni is 3 - 6 wt. The microstructure of the strip consist of >50% of fresh and tempered martensite and 5 - 20% of retained austenite, while the retained austenite carbon content is 0.5 - 1 wt %, and wherein a balance is intercritical ferrite.

## Description

### TECHNICAL FIELD

The present invention relates to 3^{rd} generation low alloyed high strength steels with excellent strength-ductility combination, and a method of manufacturing the same. In particular, the invention relates to 3^{rd} generation low alloyed high strength steels having a product of ultimate tensile strength (Rm) and total elongation (A), i.e. Rm x A, up to 50 GPa%.

### BACKGROUND OF THE INVENTION

In view of the climate change due to greenhouse gas emissions, the long-term strategy of the automotive industry is to minimize vehicle weight without compromising crash performance, affordability or product reliability. Advanced high strength steel (AHSS) products with ultimate tensile strengths of 500 - 1800 MPa are desired due to the advantage of the light weight and high strength-ductility combination, which allows for considerable reduction in automobile body weight without compromising safety requirements.

The AHSS grades can be used to make safety relevant body in white (BIW) components such as side impact protection beams in which characteristics such as capacity for energy absorption and anti-intrusion are needed in the event of a crash. The ability to absorb energy subject to loading is an essential factor to improve the impact safety of the automotive vehicles. The product of ultimate tensile strength (Rm) and total elongation (A), i.e., Rm × A, is an index of the ability to absorb impact energy. The higher the value of Rm × A, the better the ability to absorb impact energy is.

The AHSS grades are divided into three generations according to the values of Rm × A. The Rm × A is typically 10 - 25 GPa% for the first-generation AHSS including dual phase (DP) and transformation induced plasticity (TRIP) multiphase steels. The TRIP steels contain retained austenite that transforms into martensite during straining, giving the steel a combination of strength and ductility. Steels with high volume fraction of austenite also have improved wear and abrasion resistance.

The Rm × A is typically above 50 GPa% for the second-generation AHSS which is mainly represented by the high manganese twinning induced plasticity (TWIP) steels. Manganese is well known for stabilizing austenite and is therefore alloyed to produce steels with metastable retained austenite. The TWIP steels with a fully austenitic microstructure comprise manganese in the range of 15 - 25 wt.%, which inevitably results in high alloying costs and a challenging production process.

The third generation AHSS exhibits Rm × A in the range of 25 - 50 GPa% wherein the steels typically are medium manganese steels with manganese contents in the range of 3 - 10 wt.%, filling the gap between the first and second generation AHSS.

The transformation induced plasticity (TRIP) phenomenon is described as the mechanically induced martensitic transformation of metastable retained austenite. This phenomenon is important in applications where energy absorption is required, such as in vehicle crash situations. Under external loading, retained austenite transforms to fresh martensite through TRIP -mechanism during plastic deformation. This happens in gradual manner, extending uniform plastic capacity of steel matrix. When the thermal driving force, i.e. free energy for martensite transformation, is insufficient, an externally applied force can complement and trigger the transformation. The TRIP phenomenon is activated even at high deformation rates as martensite formation occurs at a rapid rate. In the absence of a competing phase transformation, retained austenite will remain in the metastable state.

Austenite Reverted Transformation (ART) annealing is a two-step heat treatment for 3^{rd} generation high strength steels. The ART annealing enables the production of steels with ultra-fine intercritical ferrite (IF), metastable retained austenite and precipitated phases. The ultra-fine intercritical ferrite (IF) is also known as high-temperature tempered martensite. The first step of the two-step heat treatment - "austenitization" - includes complete or partial austenitization followed by quenching to room temperature, resulting in a martensitic microstructure. The second step - "intercritical annealing" - reverts martensite to austenite (α' → γ), after which the steel is quenched and in some cases also tempered. The reversion (α' → γ) in the two-phase region of the initial lath martensitic microstructure allows alloying elements, such as carbon and manganese, to redistribute between intercritical ferrite (IF) and reverted austenite. It was found that carbon and substantially manganese enrichment within the volume fraction of retained austenite contribute to the chemical stabilization of retained austenite.

One major problem with the present 3^{rd} generation high strength steels is that elevated manganese alloying often leads to significant macro segregation. This may lead to deterioration of quality of the as-cast steel slab and thus the mechanical properties of the hot-rolled final product. In addition, during annealing step of the ART-treatment, diffusion coefficient of manganese is high, leading to high manganese concentration differences within the microstructure thus promoting larger ferrite phase fraction in manganese depleted areas of the final product. This too may be detrimental to the mechanical properties of the hot-rolled final product through increased heterogeneity in mechanical behavior of microstructural constituents.

### SUMMARY OF THE INVENTION

In view of the state of the art, the object of the present invention is to solve a problem of providing a hot-rolled, lean alloyed 3^{rd} generation high strength steel strip exhibiting excellent mechanical properties.

Another object of the present invention is to solve a problem of providing a hot-rolled, lean alloyed 3^{rd} generation high strength steel strip which allows for improved, wider processing window during the intercritical annealing.

Yet another object of the present invention is to solve a problem of providing a hot-rolled, low-alloyed 3^{rd} generation high strength steel having improved internal quality of the cast slab through utilizing austenite stabilizing elements having a low segregation coefficient.

These problems are solved by the combination of specific alloy design combined with an ART-heat treatment, which together result in a microstructure comprising mainly fresh and tempered martensite and finely distributed inter-lath retained austenite.

In a first aspect, the present invention provides a hot-rolled steel strip, having a yield strength of at least 600 MPa and an ultimate tensile strength of at least 1200 MPa, comprising a composition consisting of, in terms of weight percentages, wt.%:

| | |
|---|---|
| C | 0.15 - 0.4, preferably 0.18 - 0.35, more preferably 0.18 - 0.3 |

| | |
|---|---|
| Mn | 1 - 3, preferably 1.2 - 2.5, more preferably 1.5 - 2.3 |
| Si | 0 - 1, preferably 0 - 0.5, more preferably 0.1 - 0.5 |
| Al | 0.3 - 1.5, preferably, 0.4 - 1 |
| Ni | 1 - 3, preferably 1.2 - 2.8, more preferably 1.5 - 2.3 |
| Mo | 0.2 - 1, preferably 0.25 - 0.6, more preferably 0.3 - 0.5 |
| Ti | 0 - 0.2, preferably 0 - 0.1 |
| Nb | 0 - 0.1, preferably 0 - 0.1, more preferably 0 - 0.05 |
| V | 0 - 0.3, preferably 0 - 0.2, more preferably 0 - 0.1 |
| B | 0 - 0.005, |
| Ca | 0 - 0.006 |

remainder Fe and inevitable impurities, wherein

| | |
|---|---|
| P | 0 - 0.05 |
| S | 0 - 0.01 |
| N | 0 - 0.01. |

In the inventive low-alloyed steel concept, the sum of Mn and Ni is 3 - 6 wt.%, preferably 3.5 - 5 wt.% and more preferably 3.5 - 4.5 wt.%.

Furthermore, the microstructure consists of >50 % fresh and tempered martensite and 5 - 20 % retained austenite. Preferably, the microstructure consists of >80 % fresh and tempered martensite and 7 - 20 % of retained austenite. The balance is intercritical ferrite. In some embodiments, the retained austenite fraction may be 10 - 20 %. In addition, the retained austenite carbon content is 0.5 - 1 wt.% and preferably 0.5 - 0.8 wt.%.

The inventors have surprisingly found that the combination of suitable nickel and manganese alloying leads to sophisticated combination of stable and unstable austenite during the ART-annealing, after which the stable austenite remains in the final structure and unstable transforms to fresh martensite. Furthermore, the overall inventive composition design is beneficial as it allows for a wide and controllable ART-processing window allowing for precise control of austenite phase fraction, and thus, resulting in better control of mechanical properties of the final hot-rolled strip. Moreover, the lean composition allows lower ART-processing temperatures, which leads to a more energy efficient process and increased equipment service life.

Preferably, the aforementioned composition consists of, in terms of wt.%:

| | |
|---|---|
| C | 0.18 - 0.3 |
| Mn | 1.5 - 2.3 |
| Si | 0.1 - 0.5 |
| Al | 0.4 - 1 |
| Ni | 1.5 - 2 |
| Mo | 0.3 - 0.5 |
| Ti | 0 - 0.1 |
| Nb | 0 - 0.05 |
| V | 0 - 0.1 |
| B | 0 - 0.005, |
| Ca | 0 - 0.006 |

remainder Fe and inevitable impurities, wherein

| | |
|---|---|
| P | 0 - 0.05 |
| S | 0 - 0.01 |
| N | 0 - 0.01 , |

wherein the sum of Mn and Ni is 3.5 - 4.5 wt.%, and the microstructure comprise >80% of fresh and tempered martensite, and 7 - 20% of retained austenite. Furthermore, the retained austenite carbon content is 0.5 - 0.8 wt.%, and wherein a balance in the microstructure is intercritical ferrite.

Preferably, the steel exhibits a fraction of uniform elongation from a total elongation of at least 60 % and preferably 60% - 80 %. This is beneficial, as it allows maximizing energy absorption before strain localization in structural membranes.

Preferably, the steel has a microstructure comprising more than or equal to 80 %, preferably more than or equal to 90 % of fresh and tempered martensite, the reminder being retained austenite. This is beneficial, as it allows for improved strength/ductility balance and furthermore provides mechanical stability of the austenite phase during loading.

Preferably, the steel has a retained austenite fraction, measured by Electron Backscatter Diffraction (EBSD) of 0 - 1 vol.-% units from the total retained austenite fraction of 5 - 20 vol.-%, measured by X-Ray Diffraction (XRD). This is beneficial, as it ensures that the retained austenite is distributed as fine films in the microstructure as opposed to blocky retained austenite. Film-like retained austenite is more efficient in contributing to strain-induced strengthening. In other words, the film-like, finely distributed retained austenite also contributes to increased uniform elongation as opposed to blocky-like austenite that could act as a defect localizing the strain, and therefore, the benefits of retained austenite are not utilized for increased uniform elongation.

Preferably, the hot-rolled steel strip, when measured with XRD according to the description, has a face-centered cubic (FCC) (111) peak for retained austenite as part of a primary body-centered cubic (BCC) (110) peak. This is beneficial, as it indicates a finely distributed lath-like austenite morphology. Such a morphology contributes to increased uniform elongation, as discussed above.

Preferably, the hot-rolled steel strip has a yield strength (Rp0.2) in the range of 650 - 1000 MPa. Further preferably, the hot-rolled steel strip has an ultimate tensile strength (Rm) in the range of 1200 - 2000 MPa, preferably 1300 - 1800 MPa. Such a yield strength region in this strength class enables relatively low working forces during deformation process. High ultimate tensile strength, on the other hand, enables increased energy absorption prior to component failure.

Even more preferably, the hot-rolled steel strip has a yield ratio (Rp0.2/Rm) of 0.5 - 0.8. This is beneficial, as sufficient crashworthiness capability in the plastic deformation region is ensured. High strain hardening exponent ensures rapid energy absorption in the uniform elongation region thus improving crashworthiness. Furthermore, a forming process of a component is relatively easy to start, and the final component exhibits an increased yield strength due to high strain hardening exponent.

Preferably, the hardness of the hot-rolled steel strip is at least 350 HBW, preferably 350 - 500 HBW. This is beneficial, as it enables longer service life due to increased wear resistance.

In a second aspect, the present invention provides a method for manufacturing a hot-rolled steel strip comprising the following steps:
- heating a steel slab having the composition according to claim 1 to a temperature in the range of 950 °C to 1350 °C;
- hot-rolling the heated steel slab in a plurality of hot-rolling passes to produce a hot-rolled steel strip, wherein
   i) subjecting the steel slab to a plurality of hot rolling passes wherein each hot-roll pass has a predetermined temperature being either above, at or below an austenite non-recrystallization temperature in order to form a strip, wherein the final rolling temperature is in the range of 850 - 1000 °C, preferably 875 - 975 °C, and
   ii) quenching the steel strip from step (i) directly after the end of hot rolling to a cooling temperature of 350 °C or less, preferably 100 °C or less with a cooling rate of 30 - 400 °C/s, preferably 50 - 400 °C/s, more preferably 100 - 400 °C/s, and
   iii) coiling the steel strip from step (ii),
   iv) reheating the steel strip from step (iii) to an intercritical temperature in the range of A,-A₃ for a time period of 0 - 900 s, preferably 300 - 900 s, and
   v) cooling the steel strip from step (iv) to room temperature.

Preferably, the steel strip from step (iv) is cooled in air to room temperature. This is beneficial, as it is cost efficient and decreased emissions from the manufacturing process. Furthermore, air cooling is an easily repeatable process step. Air cooling enables an easy and predictable way of controlling phase distribution in the inventive alloy concept and thus affecting the resulting mechanical properties.

In a third aspect, the present invention provides a steel strip for use in manufacturing of an energy absorption component. Such components may be present in e.g. vehicles, elevators, or in other applications requiring crashworthiness.

### BRIEF DESCRIPTION OF THE DRAWINGS

Figure 1 illustrates a Gleeble thermodynamic simulation of phase transformations during an annealing process for an inventive lean alloyed steel concept.
Figures 2 a and b illustrate Gleeble A1 - A3 simulations for the inventive lean alloyed steel concept (a) and for a reference medium manganese steel (b).
Figure 3 illustrates a typical EBSD micrograph of the inventive lean alloyed steel concept.
Figures 4 a and b illustrate retained austenite morphology within a body-centered cubic (BCC) matrix in a dark field (a) and bright field (b) transmission electron microscopy (TEM) image for the inventive lean alloyed steel concept.
Figures 5 a and b illustrate typical SEM micrographs of the inventive lean alloyed steel concept (a) and reference medium manganese steel (b).
Figure 6 illustrates a typical X-ray diffraction (XRD) data set for the inventive lean alloyed steel concept.

### DETAILED DESCRIPTION OF PREFERRED EMBODIMENTS

The term "steel" is defined as an iron alloy containing carbon (C).

The symbol "A1" is used to denote the eutectoid temperature at which austenite begins to form during heating or, at which transformation of austenite to ferrite (plus cementite) is completed during cooling, where lower indices "c", "r" and "e" denote to heating, cooling and equilibrium, respectively.

The symbol "A3" is used to denote the temperature at which transformation of ferrite to austenite is completed during heating, or austenite begins to transform to ferrite during cooling, where lower indices "c", "r" and "e" denote to heating, cooling and equilibrium, respectively.

The symbol "Ms" is used to denote the temperature at which austenite begins to transform to martensite during cooling.

The symbol "ART" denotes austenite reverted transformation.

The symbol "HR" denotes hot-rolling.

The term "total elongation (A)" refers to the percentage by which the material can be stretched before it breaks; a rough indicator of formability, usually expressed as a percentage over a fixed gauge length of the measuring extensometer. Two common gauge lengths are 50 mm (A50) and 80 mm (A80).

The term "ultimate tensile strength (UTS, Rm)" refers to the point of maximum load during uniaxial tensile test. After this point, necking occurs until the final failure.

The term "yield strength (YS, Rp0.2)" refers to 0.2% offset yield strength defined as the amount of stress that will result in a plastic strain of 0.2%.

The term "heat-affected zone (HAZ)" refers to the area between the weld material and the base (unaffected) material in a welded joint.

The term body-centered cubic (BCC) refers to a unit cell structure wherein atoms are organized in a cube, with one atom in the center and one atom in each corner.

The term face-centered cubic (FCC) refers to a unit cell structure wherein atoms are organized in a cube with one atom on each side of the cube and one atom in each corner.

### Alloying elements

Alloying elements have various effects on the microstructure and mechanical properties of a hot-rolled steel strip. Thus, alloy design is one of the first issues to be considered when developing a hot-rolled steel strip with targeted mechanical properties. Alloying elements also affect the cost, processability, recyclability, weldability and coatability of steel, all of which are requirements set by the automotive industry.

Alloying elements can affect the transformation temperatures such as A1, A3 and Ms. Carbon (C), manganese (Mn) and nickel (Ni) decrease Ac1 while silicon (Si), chromium (Cr) and molybdenum (Mo) increase Ac1. Chromium (Cr) and copper (Cu) decrease Ac3 while aluminum (Al) and microalloying elements, such as niobium (Nb), titanium (Ti) and vanadium (V), increase Ac3. In commercial practice phase transformations usually occur at temperatures above the theoretical transformation temperatures determined in laboratory conditions.

Next, the chemical composition is described in more detail, wherein % of each alloying element refers to weight percentage (wt.%). Preferably, the total alloying content other than iron (Fe) is in the range of 4.5 - 8 wt.%, and more preferably 5 - 7 wt.%.

### Carbon C is used in the range of 0.15 - 0.4 %.

Carbon alloying increases the strength of the steel by solid solution strengthening, and hence C content determines the strength level of the steel. C also depresses pearlitic transformation. Furthermore, C functions as an austenite stabilizer and the austenite fraction increases by the diffusion of C into the austenite phase. C decreases A1 thereby delaying phase transformation of austenite, which inhibits the formation of ferritic-pearlitic microstructures. C content less than 0.15 % may lead to insufficient strength, and therefore, C content is preferably at least 0.18 %.

However, C has detrimental effects on e.g. weldability, weld toughness and impact toughness of steel. Therefore, C content is set to not more than 0.4 %. Preferably C is alloyed at most 0.35 % and more preferably at most 0.3 %.

### Manganese Mn is used in the range of 1 - 3 %.

Manganese is a substitutional element in the iron lattice and acts as a solid solution strengthener. There seems to be a rough relation between higher Mn content and higher strength level. Mn increases hardenability and hardness of steel and decreases the brittleness by binding to sulfur and forming manganese sulfides (MnS). Mn is a weak carbide former but a strong sulphide and oxide former. Mn also depresses pearlitic transformation.

Mn is alloyed to stabilize austenite at room temperature, i.e. the stability of austenite increases by the diffusion of Mn into the austenite phase during the intercritical annealing. In addition, Mn decreases the Ms temperature thereby delaying transformation of austenite to martensite.

Mn segregates during solidification and causes concentration gradients i.e. Mn-rich and Mn-poor regions in the microstructure. As Mn stabilizes austenite, a larger fraction of other phases than austenite is formed in the Mn-poor regions during quenching. Also, manganese decreases the chemical potential of carbon in austenite meaning that carbon diffuses from Mn-poor regions to Mn-rich regions. Consequently, austenite in Mn-rich regions receives more of stabilizing carbon during partitioning. If the carbon partitioning of austenite has been insufficient, fresh martensite forms in the Mn-rich regions during final cooling. Mn content is highest at the grain boundaries thus enabling stabilization of retained austenite in film-like morphology while the rest of the grain transforms to martensite.

Alloying with Mn more than 3 % unnecessarily increases the carbon equivalent (CE) value thereby weakening weldability. If the Mn content is too high, hardenability of the steel increases such that the heat-affect zone (HAZ) toughness is deteriorated. Large additions of Mn may also result in economic losses as manganese oxides diffuse to the slag. In addition, Mn reduces the wettability of molten Zn during galvanizing.

Preferably, Mn is used in the range of 1.2 - 2.5 %, and more preferably in the range of 1.5 -2.3%.

Furthermore, it is preferable that the steel sheet product according to the present invention has a Mn content of ≤ 10 wt.%, and more preferably in the range of 5 - 10 wt.%, within the retained austenite microstructure.

### Silicon Si is used in the range of 0 - 1 %.

Silicon is effective as a deoxidizing or killing agent and can remove oxygen from the melt during a steelmaking process. Si alloying enhances strength by solid solution strengthening, and enhances hardness by increasing austenite hardenability. Also, the presence of Si can stabilize retained austenite. Si is an effective cementite suppressor and does not form carbides. Si increases the A3 temperature of steel, meaning that the austenitization temperature increases. The presence of Si enhances stabilization of retained austenite by suppressing the formation of carbon-consuming cementite.

A Si content of higher than 1 % may cause problems during galvanizing operations, as Si may react with iron oxide and form fayalite on the hot-rolled steel surface which is difficult to remove in a pickling treatment. The rolls pick up the fayalite causing indentations on the surface of the sheet metal. Furthermore, excessive content of Si unnecessarily increases CE value thereby decreasing weldability. Silicon also promotes pearlitic transformation.

Si is preferably used in the range of 0 - 0.5% or less, and more preferably in the range of 0.1 - 0.5 %. In some embodiments, Si may be alloyed in an amount of at least 0.2 %.

### Aluminum Al is used in the range of 0.3 - 1.5%.

Aluminum is effective as a deoxidizing or killing agent and can remove oxygen from the melt during a steelmaking process. Al increases solid solution strength and hardness. Al also removes nitrogen N by forming stable aluminum nitride (AIN) particles and provides grain refinement, which promotes high toughness. Al increases the A3 temperature of steel thereby widening the austenitization temperature window. Al is an effective cementite suppressor and does not form carbides. Al stabilizes ferrite and depresses pearlitic transformation.

Al inhibits the carbon-consuming cementite precipitation thereby promoting the carbon enrichment of austenite. The stability of the austenite is determined by the balance of C and Mn, partitioned to austenite and the stabilizing effect of C is more dominant. Thus, the presence of Al can stabilize retained austenite as it allows for C to be available for partitioning to austenite instead of being bound to cementite. Al alloying also allows wider processing windows for the annealing temperature for obtaining near maximum fractions of retained austenite.

However, excess Al may increase non-metallic inclusions thereby deteriorating cleanliness of the steel. High-aluminum additions in steel deteriorate the lubrication quality and pose problems related to the function of mold flux during continuous casting of steel.

Preferably, Al is used in the range of 0.4 - 1 %.

### Nickel Ni is used in the range of 1 - 3%.

Nickel is an alloying element that decreases Ar1 thereby delaying phase transformation of austenite, which inhibits the formation of ferritic-pearlitic microstructures. Ni improves austenite hardenability thereby increasing strength without any loss of toughness. Unlike manganese, the segregation coefficient of Ni is relatively small enabling an even distribution of Ni during solidification leading to more controlled phase distribution in the final product and thus to more uniform mechanical properties.

However, Ni contents of above 3 % would increase alloying costs too much without significant technical improvement. Excess Ni may produce high viscosity iron oxide scales which deteriorate the surface quality of the hot-rolled steel strip. Higher Ni contents also have negative impacts on weldability due to increased CE value and cracking sensitivity coefficient.

Preferably Ni is alloyed in the range of 1.2 - 2.8 %, and more preferably in the range of 1.5 - 2.3 %.

### Molybdenum Mo is used in the range of 0.2 - 1%

Molybdenum is a strong solid solution strengthening element. Mo inhibits cementite formation stabilizing austenite phase. Mo also decrease the Ms temperature thus increasing hardenability. Like Ni, an even distribution of Mo during solidification due to small segregation coefficient leads to more controlled phase distribution in the final product and thus more uniform mechanical properties. Moreover, the diffusion coefficient of Mo is low in Fe lattice thus enabling uniform effect to phase stabilization during annealing. Mo is also a carbide forming element forming finely distributed carbides during tempering increasing the strength and ductility of residual tempered martensite due to precipitation strengthening. Thus, Mo alloying of at least 0.2 % is required to achieve the above mentioned effects.

However, excess alloying of Mo above 1 % would increase alloying costs too much without significant technical improvement. It would also significantly increase the CE-value, thus deteriorating the weldability of the final product.

Preferably Mo is alloyed in the range of 0.25 - 0.6 %, and more preferably in the range of 0.3 - 0.5 %.

### Niobium Nb is used in the range of 0.1% or less.

Niobium is an optional alloying element for the inventive steel concept. Nb forms niobium carbides (NbC) and carbonitrides Nb(C,N). Nb is applied as a pearlite suppressor and is a major grain refining element. Nb alloying retards recrystallization of austenite thereby impeding the grain growth. Nb alloying further stabilizes the formation of carbides thereby enabling the strengthening effects of precipitation and grain refinement.

However, only the formation of fine precipitates contribute to further grain refinement, from which precipitation strengthening may follow. Thus, large amounts of Nb do not necessarily increase the strength of the material if only higher amounts of large precipitates are formed.

Excessive content of Nb is harmful for the HAZ toughness since Nb may promote the formation of coarse upper bainite structure by forming relatively unstable TiNbN or TiNb(C,N) precipitates. Furthermore, Nb is a strong carbide stabilizing agent whereby less carbon may be available for stabilizing austenite. In case Nb is used excessively the carbon content of steel may need to be increased in order to compensate the carbon depletion due to the formation of carbides.

Therefore, the upper limit of Nb is set to 0.1 % or less, preferably 0.05 % or less.

### Vanadium V is used in the range of 0.3 % or less.

Vanadium is an optional alloying element for the inventive steel concept. V has substantially the same but smaller effects as Nb. V is a strong carbide and nitride former, but V(C,N) can also form and its solubility in austenite is higher than that of Nb or Ti. Thus, V alloying has potential for precipitation strengthening, because large quantities of V are dissolved and available for precipitation in ferrite. V alloying retards recrystallization of austenite, thereby impeding the grain growth, which leads to a fine-grained microstructure with enhanced strength. V is also applied as a pearlite suppressor. Vanadium precipitates (V4C3) in the form of plates, which enhance the resistance to hydrogen embrittlement of steel by trapping hydrogen.

However, the precipitation strengthening of V is decreased by the formation of coarse mixed compounds of microalloying elements such as (Ti,V)N. The driving force for such precipitation increases with increasing nitrogen content. Furthermore, V is a strong carbide stabilizing agent whereby less carbon may be available for stabilizing austenite. In case V is used excessively the carbon content of steel may need to be increased in order to compensate the carbon depletion due to the formation of vanadium carbides. Excessive amounts of V also have negative effects on weldability and hardenability.

Therefore, the upper limit of V is set to 0.3 % or less, preferably 0.2 % or less, more preferably 0.1 % or less.

### Titanium Ti is used in the range of 0.2 % or less.

Titanium is an optional alloying element for the inventive steel concept. Ti is applied as a grain refiner, precipitation strengthener and pearlite suppressor. Ti binds the harmful free N by forming stable titanium nitrides (TiN). TiN together with NbC can efficiently impede grain growth by retarding recrystallization of austenite, which achieves a fine-grained microstructure with enhanced strength. TiN precipitates can further prevent grain coarsening in the HAZ during welding thereby improving toughness. TiN formation also suppresses boron nitride BN precipitation, thereby leaving B free to contribute to hardenability. Furthermore, evenly distributed, relatively small, TiN particles act as excellent hydrogen traps further improving toughness. For this purpose, the ratio of Ti/N is at least 3.4.

The grain coarsening resistance is similar for steels with only TiN and Ti-rich nitrides with vanadium and niobium. Therefore, small amounts (around 0.01 %) of Ti are usually added to vanadium containing commercial steels.

However, if the Ti content is too high, coarsening of TiN and precipitation hardening due to TiC develops and the low temperature toughness may be deteriorated. Therefore, it is necessary to restrict Ti so that it is 0.2 % or less, preferably 0.1 % or less.

### Boron B is used in the range of 0.005 % or less.

Boron is an optional alloying element for the inventive steel concept. B is a well-established microalloying element added to increase hardenability. B can be added to retard phosphorus segregation to grain boundaries thereby reducing embrittlement during welding in the HAZ. Effective B alloying requires the presence of Ti to prevent formation of boron nitrides (BN). In the presence of B, Ti content can be lowered to be less than 0.02 %, which is beneficial for toughness. However, hardenability and weldability deteriorate if the B content exceeds 0.005% .

### Calcium Ca is used in a content of 0.006 % or less.

Calcium is not used as alloying element due to its low solubility in steel and high vapor pressure. The optional Ca addition during a steelmaking process is for refining, deoxidation, desulphurization, and control of shape, size and distribution of oxide and sulphide inclusions.

Unavoidable impurities can be phosphor P, sulfur S and nitrogen N. Their content in terms of weight percentages (wt.%) is preferably defined as follows:

| | |
|---|---|
| P | 0 - 0.05 |
| S | 0 - 0.01 |
| N | 0 - 0.01 |

Phosphor P suppresses the formation of cementite and acts as a solid solution strengthener. However, phosphorus decreases the hardenability of steels by forming complex phosphides that affect the amount of available substitutional elements in solid solution. Also, phosphor segregates to grain boundaries during welding in the HAZ and leads to embrittlement.

Other inevitable impurities may be hydrogen H, oxygen O and rare earth metals (REM) or the like. Their contents are limited in order to ensure excellent mechanical properties, such as impact toughness.

The steel strip product according to the present invention has a yield strength (YS) in the range of 550 - 1200 MPa, preferably 600 - 1000 MPa and a tensile strength (TS) in the range of 1200 - 2000 MPa, preferably 1300 - 1800 MPa and a yield ratio (YS/TS) in the range of 0.3 - 0.8, preferably 0.45 - 0.7. Furthermore, the minimum total A5 elongation of the steel strip product is at least 10 %.

The steel sheet product according to the present invention has a product of ultimate tensile strength (Rm) and total elongation (A), i.e. Rm x A ≤ 50 GPa%, preferably in the range of 10 GPa% to 50 GPa%.

The steel strip product according to the present invention is manufactured in a process that determines a specific microstructure which in turn dictates the above-mentioned mechanical properties of the steel sheet product.

The steel sheet product according to the present invention has a microstructure comprising >50 % of fresh and tempered martensite, preferably >80 % of fresh and tempered martensite, and 5-20 % of retained austenite, preferably 10 - 20 % of retained austenite, and the retained austenite carbon content is 0.5 - 1 wt.%, preferably 0.5 - 0.8 wt.%, wherein the balance is intercritical ferrite having spherical iron carbides.

The >50 vol.% of fresh and tempered martensite consists of tempered martensite such as high-temperature tempered martensite, and untempered martensite. Preferably, the matrix comprises ≤ 40 vol.% untempered martensite.

Carbon content of 0.5 wt.% - 1 wt.% in the retained austenite provides sufficient thermal stability for processing so that retained austenite is stable at room temperature and may thus contribute to increased elongation under plastic strain. Preferably, the matrix contains only martensite and retained austenite in the ranges disclosed above. In some embodiments, however, intercritical ferrite having spherical iron carbides may also be present in the matrix.

The steel sheet product can be provided in a wide thickness range. Preferably, the steel sheet product has a thickness of 15 mm or less, more preferably 10 mm or less, and even more preferably 6 mm or less.

### Manufacturing of a hot rolled steel strip

The method for manufacturing a hot-rolled steel strip comprise the following steps of
- providing a steel slab with a composition consisting of, in terms of weight percentages (wt.%):

| | |
|---|---|
| C | 0.15 - 0.4, preferably 0.18 - 0.35, more preferably 0.18 - 0.3 |
| Mn | 1 - 3, preferably 1.2 - 2.5, more preferably 1.5 - 2.3 |
| Si | 0 - 1, preferably 0 - 0.5, more preferably 0.1 - 0.5 |
| Al | 0.3 - 1.5, preferably, 0.4 - 1 |
| Ni | 1 - 3, preferably 1.2 - 2.8, more preferably 1.5 - 2.3 |
| Mo | 0.2 - 1, preferably 0.25 - 0.6, more preferably 0.3 - 0.5 |
| Ti | 0 - 0.2, preferably 0 - 0.1 |
| Nb | 0 - 0.1, preferably 0 - 0.1, more preferably 0 - 0.05 |
| V | 0 - 0.3, preferably 0 - 0.2, more preferably 0 - 0.1 |
| B | 0 - 0.005, |
| Ca | 0 - 0.006 |

remainder Fe and inevitable impurities, wherein

| | |
|---|---|
| P | 0 - 0.05 |
| S | 0 - 0.01 |
| N | 0 - 0.01 , |

remainder Fe and inevitable impurities;
- heating said steel slab to a temperature in the range of 950 - 1350 °C;
- hot-rolling the heated steel slab in a plurality of hot-rolling passes to produce a hot-rolled steel strip, wherein
i) subjecting the steel slab to a plurality of hot-rolling passes wherein each hot-roll pass has a predetermined temperature being either above, at or below an austenite non-recrystallization temperature in order to form a strip, wherein the final rolling temperature is in the range of 850 - 1000 °C, preferably 875 - 975 °C, and
ii) quenching the steel strip from step (i) directly after the end of hot rolling to a cooling temperature of 350 °C or less, preferably 100 °C or less with a cooling rate of 30 - 400 °C/s, preferably 50 - 400 °C/s, more preferably 100 - 400 °C/s, and
iii) coiling the steel strip from step (ii),
iv) reheating the steel strip from step (iii) to an intercritical temperature in the range of A,-A₃ for a time period of 0 - 900 s, preferably 300 - 900 s, and
v) cooling the steel strip from step (iv) to room temperature.

The step of intercritical annealing (iv) may be performed e.g. by batch annealing or continuous annealing.

In some embodiments, the final step of cooling to room temperature (v) is continuous cooling. Optionally, the step of cooling to room temperature is followed by a heat treatment at a temperature in the range of 200 - 400 °C for a time period in the range of 30 - 200 seconds, preferably around 100 seconds. In such an embodiment, bainitic and/or martensitic transformations may occur to some degree during the step of final cooling to room temperature (v), which result in volume fractions of bainite and fresh untempered martensite in the final microstructure. The heat treatment at a temperature in the range of 200 - 400 °C facilitates formation of the tempered martensite. Due to carbide precipitation the heat treatment decreases the tensile strength while increasing the yield strength.

In another embodiment, the step of final cooling to room temperature (v) comprises the following steps:
- cooling the steel strip in a first cooling step to an annealing temperature in the range of 430 - 530 °C;
- annealing at a temperature in the range of 430 - 530 °C for a time period in the range of 30 - 200 seconds; and
- cooling the annealed steel strip in a second cooling step to room temperature.

In such an embodiment, the annealing at a temperature in the range of 430 - 530 °C is effectively a partitioning annealing, which enables stabilization of reverted austenite to room temperature by enriching carbon within the reverted austenite. Preferably, the time period of annealing at a temperature in the range of 430 - 530 °C is around 100 seconds.

In yet another embodiment, the step of final cooling to room temperature (v) comprises the following steps:
- cooling the steel strip in a first cooling the steel to a temperature below the Ms temperature;
- holding the steel strip at constant temperature for a time of 10 - 300 s;
- cooling the steel strip in a second cooling step to room temperature.

Traditionally, medium manganese steels have been based on the design idea of alloying with increased manganese content in order to allow stabilization of retained austenite during intercritical annealing through diffusion of manganese. Diffusion control of alloying elements to retained austenite during intercritical annealing at high temperatures (around A3 temperature) is difficult, as diffusion flux of elements, such as manganese, increases drastically with increasing temperature.

Previous studies suggested that blocky austenite nucleates at prior austenite grain (PAG) boundaries whereas lath-like austenite forms between martensite laths during the intercritical annealing. The lath-like austenite is more easily enriched with the austenite stabilizing carbon than the blocky austenite. A martensitic microstructure is considered an ideal starting point for the intercritical annealing process step in the aforementioned method according to the present invention. This is because the martensite phase prior to intercritical annealing step enhances the formation of lath-like austenite. The newly formed lath-like austenite is easily enriched with austenite stabilizing carbon. Diffusion of manganese to high-angle boundaries, such as grain boundaries and martensite packet boundaries, further stabilizes austenite phase so that lath-like austenite remains in the fresh martensite matrix after cooling to room temperature. This ensures that the retained austenite morphology is finely dispersed lath-like austenite instead of blocky-like austenite. Lath-like austenite is mechanically stable and thus enhances elongation properties during plastic strain.

In the present inventive steel concept, however, part of manganese alloying has been replaced with nickel, which is an effective FCC phase stabilizer and has a small diffusion coefficient. Furthermore, during the intercritical annealing, manganese diffuses to austenite (an FCC phase) thus increasing the stability of retained austenite at room temperature. During the intercritical annealing, manganese, nickel and carbon together enable for stabilization of freshly formed austenite, part of which then transforms to fresh martensite during the final cooling step to room temperature. The diffusion of manganese to high-angle boundaries such as grain boundaries locally stabilizes austenite phase while the core of the austenite grains formed during the intercritical annealing transforms to fresh martensite during the final cooling to room temperature. This mechanism enables formation of new microstructure consisting of fresh martensite and nanoscale inter-lath retained austenite, which provides, together with existing tempered martensite, excellent mechanical properties.

Figure 1 illustrates a Gleeble thermodynamic simulation of phase transformations during an annealing process for an inventive lean alloyed steel concept. The solid line in Figure 1 denotes heating data and dashed line denotes cooling data. In the simulation, the annealing temperature used was 740 °C with a dwell time of 600 s followed by air-cooling. From Figure 1, it can be seen that only martensite transformation was detected during the cooling phase.

Figures 2 a and b illustrate Gleeble A1-A3 simulations for the inventive lean alloyed steel concept (a) and for a reference medium manganese steel (b). In both Figures, A1_{JMP} denotes to a calculated A1 temperature using J-Mat Pro^{™} software, and A1_{G} and A3 denote to the A1 and A3 temperatures, respectively, determined by Gleeble simulation.

Figure 2a shows that the Gleeble sample of the inventive lean alloy steel concept exhibits a linear increase of an austenite phase fraction with increasing temperature between A1 and A3. This is beneficial for process control as temperature-time relation can be predicted more easily. Furthermore, intercritical annealing temperatures are lower for the inventive steel sample allowing energy savings and longer service life of process equipment. Meanwhile, Figure 2b shows that the reference medium manganese steel sample exhibits non-linear behavior that is detrimental for predicting phase constituents in the final product.

The following Examples further describe and demonstrate embodiments within the scope of the present invention. The Examples are given solely for the purpose of illustration and are not to be construed as limitations of the present invention, as many variations thereof are possible without departing from the scope of the invention.

### EXAMPLES

### Composition

Table 1 shows the chemical compositions of the tested steels. Compared to the reference sample, the inventive steel concept sample has lower Mn, Si and Al content and increased Ni and Mo contents. In the inventive steel concept, Mn content has been decreased in order to reduce the severity of macro segregation. Precipitation kinetics have been modified by Mo alloying to suppress cementite formation prior to A1 temperature. To compensate lack of FCC phase stabilization, Mn alloying has been partly replaced with Ni alloying to achieve sufficient FCC phase stability, as Ni leads to a reduced level of macro segregation. Decreased levels of Si and Al help to keep the overall alloying amount on a reasonable level. Reduced Si also helps to promote better surface quality. Optional alloying elements were not purposefully alloyed to the Examples herein, but some trace levels of such elements, e.g. Ti, Nb or V, may be present.

### Manufacturing method

Both samples were rolled using a laboratory rolling mill and furnaces. The processing parameters for both the inventive steel concept and the reference steel are shown in Table 2. Both samples were first austenitized, then hot-rolled and quenched to room temperature. At this stage, the microstructure of the steels was fully martensitic. This is a beneficial starting microstructure for the ART-annealing cycle, because the martensitic starting microstructure prior to the step of intercritical annealing enhances the formation of acicular or lath-like austenite, which is more easily enriched by carbon as opposed to blocky austenite morphology.

The ART-annealing temperature was selected so that the microstructure of the steel contained some fraction of austenite and intercritical ferrite at the annealing temperature. During the ART-annealing, carbon in solution is diffused to austenite thus enabling stabilization of austenite at room temperature after the final cooling to room temperature. Both samples were cooled in air to room temperature after the ART-annealing.

### Microstructures

Phase fraction data and austenite carbon content in the final microstructure is shown in Table 3. Microstructures of the studied samples were characterized using Scanning Electron Microscopy (SEM) and Electron Back-Scatter Diffraction (EBSD) and the volume fraction of retained austenite was determined by using both EBSD as well as X-ray diffraction (XRD). Austenite carbon content was calculated from XRD data using the following equation: $a γ = 3.556 + 0.0453 \times C + 0.00095 \times Mn + 0.0056 \times Al - 0.0002 \times Ni + 0.0031 \times Mo + 0.0017 \times V$ where aγ is the austenite lattice parameter (Å) and xC, xMn, xAl, xNi, xMo and xV are the concentrations (in wt.%) of C, Mn, Al, Ni, Mo and V, respectively.

EBSD analysis was conducted with JEOL JSM-7900F FESEM equipped with Oxford Instruments Aztec -software. Step size for EBSD measurements was 0.05 µm with a magnification of x2000, a working distance of 10 mm and an acceleration voltage of 15 keV. Sample orientation was RD-TD and the measurement surface was electrolytically polished.

XRD measurements were conducted for the EBSD specimens on a Rigaku SmartLab X-Ray Diffractometer (XRD) with a 5.4 kW Co radiation source and a CBO-f polycapillary x-ray optics was used in the XRD data acquisition. The data was analyzed using PDXL2 software. The step size of 0.01° and the scan speed 0.5°/60 s over the 2-**θ** range of 45-130° were used in the measurements. The achieved data was used to estimate the specimens' lattice parameters of austenite in the electrolytic etched specimens. The fundamental parameter (FP) method of the PDXL2 analysis software was used to calculate the specimens' lattice parameters of the retained austenite by using whole powder pattern decomposition method (WPPD) of the software.

The volume fraction of retained austenite (RA) was measured by using Rietveld whole powder pattern fitting method (WPPF) of the analysis software. The effect of texture on the relative peak intensities in the diffractograms was reduced by a detexturizing procedure during the measurements. This improved the accuracy of the RA phase volume fraction estimation. In this procedure, seven diffraction scans are taken while the specimen was tilted at ten-degree intervals from 0 - 60 ° along the x axis of the Euler cradle and simultaneously rotated 360° along the **ϕ**-axis. Afterwards, an average diffractogram is created from the measured diffractograms for the WPPF analysis. The adverse effect of defocusing on the quality of the diffractogram was minimized by using focused X-Ray optics.

Table 3 shows that retained austenite fraction is significantly greater when measured with XRD as opposed to the values obtained by EBSD. This indicates that the majority of the retained austenite is of finely distributed, lath-like morphology. Furthermore, Table 3 illustrates that in the reference steel, a higher fraction of the retained austenite is present in a blocky morphology. This is evident from the fact that the retained austenite fraction measured with EBSD is greater in the reference steel. Table 3 also shows that the carbon content in the retained austenite in the inventive steel is greater than in the reference steel.

Figure 3 illustrates a typical band-contrast micrograph of the inventive steel captured with EBSD. Darker color in Figure 3 indicates higher dislocation density in the vicinity of fresh martensite. Figure 3 shows that the microstructure comprises tempered martensite (TM), fresh martensite (FM) and globular (blocky) retained austenite. The finely distributed, lath-like retained austenite is not distinguishable from this EBSD micrograph. As can be seen from Figure 3, the fraction of blocky retained austenite is low in the final microstructure. The phase fraction of retained austenite in this micrograph is 0.1 % as detected by EBSD.

Figures 4 a and b illustrate retained austenite morphology within a BCC matrix in a dark field (a) and bright field (b) transmission electron microscopy (TEM) image pair. The side figure on the top-left corner of Figure 4a shows the Kurdjumov-Sachs (K-S) relation between the BCC and FCC phases. Figure 4 further illustrates the fact that the retained austenite that is present in the microstructure is of fine, lath-like morphology.

Figures 5 a and b illustrate typical SEM micrographs of the inventive steel (a) and reference steel (b). Figure 5a shows that the sizes of microstructure constituents are smaller in the inventive steel concept, which indicates a more uniform austenite nucleation during intercritical annealing.

Figure 6 illustrates a typical XRD data set for the inventive steel concept. Here, it is shown that the austenite peak (FCC) is part of the ferrite peak (BCC), since the intensity does not drop between the FCC (111) peak and BCC (110) peaks. This in turn indicates that the austenite phase is distributed as fine, lath-like structures within the ferrite matrix and not as a separate blocky phase, as also seen in Figure 4a.

### Mechanical properties

Tensile properties were determined according to SFS-EN ISO 6892-1:2019 using a sample having the following dimensions: nominal width 12.5 mm, gauge length 50 mm, parallel length 75 mm, width of the grip end 20 mm, length of the grip end 75 mm and radius 12 mm. Table 4 illustrates that the inventive lean alloyed steel concept sample has a greater yield strength and total elongation with a comparable ultimate tensile strength level than the reference medium manganese steel. As seen from Figure 5a and Table 4, finer distribution of microstructure constituents results in a more homogenic mechanical behavior resulting in improved ductility, and thus improved total elongation, for the inventive lean alloyed steel concept. Furthermore, the inventive lean alloyed steel concept sample exhibits greater uniform elongation level indicating more homogenous microstructure and improved distribution of stresses during plastic deformation. Table 4 also shows HV10 hardness values measured for the Examples. Hardness measurements were conducted according to SFS EN-ISO 6507-1 standard. Both the inventive lean alloyed steel concept and the reference medium manganese steel exhibit similar hardness values.

**Table 1**

| Example | C | Mn | Si | Al | Ni | Mo |
|---|---|---|---|---|---|---|
| 1 (INV) | 0.2 | 1.87 | 0.31 | 0.53 | 1.66 | 0.41 |
| 2 (REF) | 0.2 | 3.37 | 0.96 | 1.5 | 0.97 | 0.21 |

**Table 2**

| Example | AT (°C) | FRT (°C) | CT1 (°C) | CR1 (°C/s) | ART (°C) | CT (°C) | CR2 (°C/s) |
|---|---|---|---|---|---|---|---|
| 1 (INV) | 1100 | 930 | 25 | 100 | 740 | 25 | 5 |
| 2 (COMP) | 1100 | 924 | 25 | 100 | 790 | 25 | 5 |

**Table 3**

| Example | M -% | EBSD RA -% | XRD RA -% | RA C -% | INT BCC -% |
|---|---|---|---|---|---|
| 1 (INV) | 83 | 0.2 | 8 | 0.71 | 9 |
| 2 (COMP) | 75 | 1.2 | 10 | 0.62 | 15 |

**Table 4**

| Example | YS (MPa) | UTS (MPa) | YR (%) | UE (%) | TE (%) | UTS*TE (MPa*%) | HV10 (kgf/mm²) |
|---|---|---|---|---|---|---|---|
| 1 (INV) | 739 | 1417 | 0.52 | 9.4 | 13.2 | 18700 | 378 |
| 2 (COMP) | 687 | 1459 | 0.47 | 7.5 | 9.1 | 13276 | 375 |

## Claims

1. A hot-rolled steel strip, having a yield strength of at least 600 MPa and an ultimate tensile strength of at least 1200 MPa, comprising a composition consisting of, in terms of weight percentages, wt.%:
| | |
|---|---|
| C | 0.15 - 0.4 |
| Mn | 1 - 3 |
| Si | 0 - 1 |
| Al | 0.3 - 1.5 |
| Ni | 1 - 3 |
| Mo | 0.2 - 1 |
| Ti | 0 - 0.2 |
| Nb | 0 - 0.1 |
| V | 0 - 0.3 |
| B | 0 - 0.005 |
| Ca | 0 - 0.006 |
remainder Fe and inevitable impurities, wherein
| | |
|---|---|
| P | 0 - 0.05 |
| S | 0 - 0.01 |
| N | 0 - 0.01 , |
and wherein
the sum of Mn and Ni is 3 - 6 wt, and
the microstructure consist of >50% of fresh and tempered martensite, and 5 - 20% of retained austenite, and
the retained austenite carbon content is 0.5 - 1 wt.%,
and wherein a balance is intercritical ferrite.

2. The hot-rolled steel strip according to claim 1, wherein
the C content is 0.18 - 0.35 wt.% and preferably 0.18 - 0.3 wt.%.

3. The hot-rolled steel strip according any one of the preceding claims, wherein the Mn content is 1.2 - 2.5 wt.% and preferably 1.5 - 2.3 wt.%.

4. The hot-rolled steel strip according any one of the preceding claims, wherein the Si content is 0 - 0.5 wt.% and preferably 0.1 - 0.5 wt.%.

5. The hot-rolled steel strip according any one of the preceding claims, wherein the Al content is 0.4 - 1 wt.%.

6. The hot-rolled steel strip according any one of the preceding claims, wherein the Ni content is 1.2 - 2.8 wt.% and preferably 1.5 - 2.3 wt.%.

7. The hot-rolled steel strip according any one of the preceding claims, wherein the Mo content is 0.25 - 0.6 wt.% and preferably 0.3 - 0.5 wt.%.

8. The hot-rolled steel strip according any one of the preceding claims, wherein the sum of Mn and Ni is 3 - 6 wt.%, preferably 3.5 - 5 wt.% and more preferably 3.5 - 4.5 wt.%

9. The hot-rolled steel strip according any one of the preceding claims, wherein the fraction of uniform elongation from total elongation is at least 60% and preferably 60% - 80%.

10. The hot-rolled steel strip according any one of the preceding claims having a microstructure consisting >80 % of fresh and tempered martensite and 7 - 20 % of retained austenite, the reminder being intercritical ferrite, wherein
the retained austenite carbon content is 0.5 - 0.8 wt.%.

11. The hot-rolled steel strip according claim 10, having
a microstructure consisting of more than or equal to 80% of, preferably 90% of fresh and tempered martensite, the reminder being retained austenite, wherein the retained austenite carbon content is 0.5 - 0.8 wt.%.

12. The hot-rolled steel strip according any one of the preceding claims, having a retained austenite fraction, measured by EBSD according to description, of 0 - 1 vol.-% units from the total retained austenite fraction of 5 - 20 vol.-%, measured by XRD according to the description.

13. The hot-rolled steel strip according any one of the preceding claims, wherein, when measured with XRD according to the description, a face-centered cubic (FCC) (111) peak for retained austenite is part of a primary body-centered cubic (BCC) (110) peak.

14. A method for manufacturing a hot-rolled steel strip according to claims 1-13 comprising the following steps of
- heating a steel slab having a following composition:
| | |
|---|---|
| C | 0.15 - 0.4 |
| Mn | 1 - 3 |
| Si | 0 - 1 |
| Al | 0.3 - 1.5 |
| Ni | 1 - 3 |
| Mo | 0.2 - 1 |
| Ti | 0 - 0.2 |
| Nb | 0 - 0.1 |
| V | 0 - 0.3 |
| B | 0 - 0.005 |
| Ca | 0 - 0.006 |
remainder Fe and inevitable impurities, wherein
| | |
|---|---|
| P | 0 - 0.05 |
| S | 0 - 0.01 |
| N | 0 - 0.01 , |
and wherein the sum of Mn and Ni is 3 - 6 wt, to a temperature in the range of 950 °C to 1350 °C;
- hot rolling the heated steel slab in a plurality of hot rolling passes to produce a hot rolled steel strip, wherein
i) subjecting the steel slab to a plurality of hot rolling passes, wherein each hot-roll pass has a predetermined temperature being either above, at, or below an austenite non-recrystallization temperature in order to form a strip, wherein the final rolling temperature is in the range of 850 - 1000 °C, preferably 875 - 975 °C, and
ii) quenching the steel strip from step (i) directly after the end of hot rolling to a cooling temperature of 350 °C or less, preferably 100 °C or less with a cooling rate of 30 - 400 °C/s, preferably 50 - 400 °C/s, more preferably 100 - 400 °C/s, and
iii) coiling the steel strip from step (ii),
iv) reheating the steel strip from step (iii) to an intercritical temperature in the range of A₁-A₃ for a time period of 0 - 900 s, preferably 300 - 900 s, and
v) cooling the steel strip from step (iv) to room temperature.

15. The method for manufacturing a steel strip according to claim 14, wherein,
- the steel strip from step (iv) is cooled in air to room temperature.
